

J. C. HARTOGS.  
MANUFACTURE OF ARTIFICIAL THREAD.  
APPLICATION FILED JULY 26, 1911.

1,119,155.

Patented Dec. 1, 1914.



Witnesses

N. P. Leonard.  
N. E. Costello.

Jacques Coenraad Hartogs  
Inventor

By  
Bynes, Fowles & Brickestein

Attorneys

# UNITED STATES PATENT OFFICE

JACQUES COENRAAD HARTOGS, OF AMSTERDAM, NETHERLANDS, ASSIGNOR TO N. V.  
NEDERLANDSCHE KUNSTZIJDEFABRIEK, OF VOSDIJK ARNHEM, NETHERLANDS,  
INCORPORATED.

## MANUFACTURE OF ARTIFICIAL THREAD.

1,119,155.

Specification of Letters Patent.

Patented Dec. 1, 1914.

Application filed July 26, 1911. Serial No. 640,660.

To all whom it may concern:

Be it known that I, JACQUES COENRAAD HARTOGS, subject of the Queen of the Netherlands, residing at No. 15 Alexanderkade, 5 Amsterdam, Province of North Holland, Netherlands, have invented certain new and useful Improvements in the Manufacture of Artificial Thread, of which the following is a specification.

10 This invention relates to a process for the manufacture of artificial thread and is especially suitable for the manufacture of artificial silk from cellulose or its derivatives or from solutions of casein, fibroin, viscose 15 or the like.

In the manufacture of artificial thread especially artificial silk, several points must be considered, viz. the coagulation of the fluid, the fixing of the coagulated mass, the 20 preservation of the softness of the finished thread and the prevention of the sticking together of the separate threads. Hitherto it has been sought to effect these objects either by the use of a single bath fulfilling 25 all the conditions or especially when spinning artificial silk by the use of several baths. According to this invention I effect these four objects without the use of different vessels for the reception of the different 30 liquids by the employment of different liquids which are little if at all miscible with each other. Preferably I employ liquids of different density which form superposed layers. For example threads of cellulose 35 may first be coagulated in an aqueous fluid, and then led in such a manner that the spun fibers do not touch each other for further treatment through a fluid of different density such for example as benzene, oil, nitro- 40 benzene, chloroform, carbon tetrachlorid, or the like, where they receive a thin coating, which prevents them from sticking together when they are combined into a thicker thread. If desired the threads may again 45 pass through the same aqueous layer and also if desired through a liquid floating upon the aqueous liquid.

In the accompanying drawings Figures 1, 2 and 3 show diagrammatically three methods of carrying out the invention.

50 *a* is the vessel containing the viscous liquid and *b* are its spinning nozzles from which separate threads *c* issue to be combined later into a single thread *c'*.

55 In Fig. 1 *d* is an aqueous liquid such as a

dilute acid for example and *e* is a layer of benzene, oil or other organic liquid which floats upon the layer *d*. While passing through the layer *e* the separate fibers *c* receive a thin coating of an indifferent liquid, 60 which prevents them from sticking together when they are combined into a stouter thread *c'*. The aqueous liquid *d* may be made of high specific gravity by dissolving in it some inert salt, glycerin or the like. 65 Its density may be decreased by admixture with a suitable body such as alcohol, acetone or the like.

In Fig. 2, *f* is an aqueous liquid which coagulates the separate threads *c* issuing 70 from the spinning nozzles *b*. *g* is a second heavier liquid such for example as nitrobenzene, chloroform, carbon tetrachlorid or the like lying beneath the layer *f* through which the separate fibers pass. The fibers *c* 75 may be combined into a single thread in this fluid in any suitable manner but preferably the threads are then reversed in direction by passing beneath a rod *r* (or other equivalent arrangement) located in the bottom of 80 the vessel; they will in this case again pass through the aqueous liquid *f* thus preventing the threads from sticking together in consequence of the thin coating received by 85 their passage through the liquid *g*.

In Fig. 3 *h* is an aqueous liquid, *i* is a liquid heavier than *h* such as nitrobenzene, chloroform, carbon tetrachlorid or like heavy liquid, *k* is a liquid such as benzene, ether or the like which floats upon the 90 liquid *h*.

The separate threads *c* coagulate in their passage through the liquid *h* and then pass through the liquid *i* in which they are combined to a single thread *c'*; they then pass 95 beneath a rod *r* or its equivalent and return through the liquid *h* and through the liquid *k* which serves to wash them.

The invention is eminently adapted for spinning a good artificial silk from solutions of viscose in dilute sulfuric acid without other addition which has hitherto been impossible.

The process may be carried out in the apparatus shown in Fig. 1 the liquid *d* consisting of dilute sulfuric acid and the liquid *e* of an oil. The separate threads are after their passage through the spinning bath *d* and the coating fluid *e* left for some time to themselves thus allowing them to be 110

thoroughly fixed without the possibility of their sticking together.

The coating of oil or the like can be removed from the threads for example by 5 washing in a 1% soda solution or some organic solvent such as benzene. The product so obtained excels others heretofore produced.

What I claim is:

19 1. The process of making artificial thread in one bath, which comprises coagulating separate filaments of dissolved cellulose issued through fine orifices by passing the same through a decomposing solution which 15 acts quickly on the cellulose solution, then coating the completely coagulated separate filaments to make them non-sticking by passing them through an indifferent liquid, then combining the coagulated non-sticking 20 separate filaments into a thread.

2. The process of making artificial thread in one bath, which comprises coagulating separate filaments of dissolved cellulose issued through fine orifices by passing the same through a decomposing solution which 25 acts quickly on the cellulose solution, preventing the completely coagulated separate

filaments from sticking by then passing them through a contacting layer of an indifferent liquid whereby a coating of said 30 indifferent liquid envelops the separate filaments, then combining the coagulated coated separate filaments into a thread.

3. The process of making artificial thread in one bath, which comprises coagulating 35 separate filaments of dissolved cellulose issued through fine orifices by passing the same through a decomposing solution which acts quickly on the cellulose solution, preventing the completely coagulated separate 40 filaments from sticking by then passing them through a contacting layer of an indifferent liquid whereby a coating of said 45 indifferent liquid envelops the separate filaments, combining the coagulated coated separated filaments into a thread, then washing the thread.

In testimony whereof I have hereunto set my hand in presence of two subscribing witnesses.

JACQUES COENRAAD HARTOGS.

Witnesses:

THOMAS H. VERHAVE,  
D. P. DE YOUNG.